

## 1

3,173,841

**DURABLE ANTIBACTERIAL TEXTILE FINISH  
FOR CELLULOSIC TEXTILE MATERIAL**

Philip B. Roth, Somerville, N.J., and Leonard B. Hallows, Lima, Peru, assignors to American Cyanamid Company, Stamford, Conn., a corporation of Maine  
No Drawing. Filed Aug. 23, 1962, Ser. No. 218,851  
8 Claims. (Cl. 167—84)

This invention relates to durable antibacterial finishes for textile materials in which the active antibacterial agent is neomycin, to methods for applying the same to textile materials, and to the materials so treated.

In recent years, increased attention has been given to the development of textile finishes of this type, which have become known as purifying finishes. These finishes are intended to reduce the number of microorganisms residing in the materials, whereby such materials may be used with less danger from harmful bacteria. These purifying finishes, when applied to articles of clothing worn close to the body, are also helpful in the prevention of the development of odor.

A satisfactory purifying finish should be durable and active at low concentrations against a broad spectrum of microorganisms. It should be non-toxic and non-allergenic. It should not have the tendency to sensitize the wearer of the textile material to the material to be finished. It should not have the quality of allowing strains of bacteria to develop, which are resistant to the antibacterial agent of the finish. Still further, it should be resistant to home and commercial laundering conditions and should impart little or no modification of the hand of the textile.

Neomycin employed as a purifying finish is highly satisfactory with respect to most of the categories mentioned above, and its use is described fully in U.S. Patent No. 2,830,011, the subject matter of which is incorporated herein by reference. The finish imparted by neomycin employed in accordance with the disclosure of the above referred to U.S. patent, insofar as textile materials containing cellulosic fibers are concerned, provides a satisfactory and durable finish, which remains antibacterial after numerous launderings. This durability is believed to be the result of the neomycin being substantive to the cellulose base material.

While the treatment of cellulosic fibers with neomycin in accordance with the above referred to patent imparts excellent antibacterial properties which remain after the cleaning or processing of the fiber or fabric formed therefrom, the washing of neomycin treated fabrics, particularly in hard water, with soap, causes the fibers to become yellowish and dull in appearance. This yellowishness or dullness apparently is the result of the formation of neomycin stearate or a mixed salt of calcium or magnesium and neomycin with stearic acid, when finished fabrics are laundered with soap. While laundering with soaps increases the yellowness or dullness of neomycin finished fabric, laundering with other cleaning agents, as for example, detergents, will also result in yellowing of the finished fabric, although to a lesser degree and at a more gradual rate. The yellowing effect is, of course, very undesirable and any agent or procedure which will minimize or conceal the development of color or dullness is of great importance in the commercialization of neomycin as a purifying finish.

While it may be assumed that the yellowing or dullness appearing in neomycin treated fabrics that have been laundered can be corrected by the employment of chemical bleaches, such is not the case. This is true in that in most instances the use of such bleaches, as for example, those containing chlorine, functions to destroy the antibacterial activity of the neomycin.

## 2

For many years it has been the practice to attempt to conceal the yellowish cast of cellulosic materials by the use of blue pigments or dyes, that is, to neutralize the yellow color of the cellulosic material by adding the complementary color, blue. For this purpose, the use of blue pigments, such as ultramarine or alkali blue or of fugitive blue dyestuffs has long been common practice in fabric and paper manufacture and in laundering operations.

10 While these blue coloring materials are often temporarily effective, they are subject to series disadvantages. For example, the addition of a blue color to a yellow does not produce a pure white, but rather a gray, because both colors are absorbing light and reducing the 15 total amount of reflected light. Further, unless the exact coloring balance is struck, the finished product is not even a gray, but actually may be blue.

Accordingly, it is an object of the present invention to provide a process whereby neomycin as an antibacterial agent may be imparted by a single application step to a textile material containing cellulose, so that the material, when laundered, is substantially free from yellowness and/or dullness, which is characteristic of laundered neomycin finished cellulose containing textile materials.

20 A further object of the present invention is to provide such a process which does not interfere with the antibacterial activity of the neomycin on the fabric, and one which may be accomplished employing conventional 25 finishing equipment and known chemical materials.

It is a further object of the present invention to provide neomycin finished cellulose containing textile materials, which upon repeated launderings manifest substantial improvement with respect to less yellowing and dullness, normally associated with such materials finished 30 in accordance with the prior art procedures.

Another object of this invention is to provide novel 35 stable compositions of matter containing neomycin as an antibacterial agent, which when imparted onto cellulose containing textile material by a single application step, yellow less and are less dull than those finishes in accordance with prior art procedures.

These and other objects and advantages of the present 40 invention will appear more clearly from the detailed description thereof set forth hereinbelow.

It has been discovered in accordance with the present 45 invention that the discoloration or staining (yellowishness or dullness) caused by the laundering or washing of neomycin treated cellulosic textile materials or cellulose containing textile materials can be prevented or at 50 least largely concealed by applying in a single application step anionic fluorescent textile brighteners (optical bleaches) and neomycin from stable aqueous solutions containing the same. It will be apparent that the neomycin 55 and brightener must be applied in effective amounts. The stable solutions containing the anionic brighteners and neomycin, to be discussed more fully hereinafter, constitute an essential element of this invention. In view of the fact that neomycin is a cationic material, it will be 60 appreciated that the introduction of such material into an aqueous solution of anionic brightener or vice versa produces a precipitate. Such compositions or suspensions are not suitable for use in conventional application procedures, due to the fact that good quality control is 65 most difficult to maintain when they are employed.

In overcoming this difficulty, we have discovered that if the pH of aqueous solution containing neomycin and a suitable anionic brightener is above 8, these materials are rendered compatible and may be applied in a single 70 application step.

Since most neomycin solutions are acidic, usually a pH of less than 3 and normally a pH of from about 1

to about 2, even the addition of alkaline brightener solution rarely raises the pH more than a few units, because of the small amounts of brightener employed. Thus adjustment from the acid side to a pH value above 8 is effected with suitable alkaline agents such as sodium hydroxide, potassium hydroxide, sodium carbonate, potassium carbonate, ammonia, organic amines and their equivalents.

While the pH of the solution should be above 8, we have found that as a practical matter the pH of the treating solution should be above 8.5 and is normally about 9. The pH can certainly be higher than 9, as for example 10, 11 or more, but addition of amounts of base which are more than sufficient to produce clear stable aqueous solutions of neomycin and brightener is unnecessary and undesirable in the light of economic considerations.

To prepare a suitable stable solution, solutions of the components may be mixed and the pH adjusted or suitable base may be added to either or both components prior to mixing. If the components are first mixed, the precipitate that is formed and is evidenced initially by a haze or cloudiness in the solution, may be removed by the

the spectrum, thereby compensating for the slightly yellowish cast of most white fabrics.

Suitable brighteners for use in this invention may be divided into two types, according to the type of fiber for which they have affinity. There are the cellulosic and all-purpose types, the latter having affinity for both cellulosic and non-cellulosic fibers. Since this invention is restricted to application of solutions to textile materials containing cellulosic fibers, only such brighteners are contemplated.

Such brighteners may also be divided into chemical classes. The members of the cellulosic type can, for the most part, be assigned to the following classes: acyldiaminostilbene (I), triazinylaminostilbenes (II), and acyldiaminodibenzothiophene dioxides (III). The members of these classes contain sulfonic acid groups. The "all-purpose" type comprises the benzimidazoles (IV) and the triazoles (V). Only those members of classes IV and V containing one or more sulfonic acid groups are contemplated for use in the instant invention.

Typical general formulae for classes I-III are illustrated below:



addition of base to the pH value above 8.5 as indicated above. Regardless of how the final solution having such a pH is produced, the essential point is that the solution have such a final pH value.

It should be noted that the term "neomycin" is used herein in its ordinary sense, and as it is defined in U.S. Patent No. 2,830,011, above referred to. In general, this refers to a commercially available product which is called neomycin, which is actually a mixture of two very closely related antibiotics known more specifically as neomycin B and neomycin C. The term is also intended to cover neomycin as just defined, the individual components of the complex, or its salts, of which the sulfate is the most generally available. Other salts of neomycin have been used in finishing textiles with good results, among them may be mentioned neomycin parahydroxybenzoate, neomycin sulfanilate, neomycin-N-tartrate, neomycin propionate, neomycin aconitate, neomycin phthalate, neomycin undecylinate, neomycin palmitate, neomycin stearate, and others.

By "cellulosic textile materials" or "cellulose containing textile materials," as these terms are employed herein, it is meant fibers or formed fabrics, either woven or felted, containing at least 50% fibers of cellulosic origin and preferably composed entirely of cellulose for maximum effect. As examples of cellulosic textile materials, the following are illustrative: cotton, regenerated cellulose, linen, jute, hemp, and the like. Blends of these materials and combinations of these materials or blends thereof with wool, silk, nylon, acrylic fibers, polyester fibers, and the like, are also contemplated.

The use of fluorescent textile brighteners or "optical bleaches" in general fields of application represent advancement over prior art techniques attempting to conceal the yellowish cast on cellulosic materials which employed blue pigments or dyes. Thus, instead of using a blue pigment, which absorbs colored light in the yellow range, their use involves the employment of a fluorescent substance, which emits colored light in the blue range. Thus, the yellowing effect is destroyed by a substance which emits the blue light.

In recent years, the use of these optical bleaching agents or brighteners has grown enormously. These compositions are colorless dyestuffs, exhibiting affinity for fabrics, which when exposed to ultraviolet radiation, such as is contained in day light, fluoresce in the blue range of

45 wherein R, R', R'' and R''', by way of example, may be hydrogen, alkyl, aryl, alkoxy, halogen, nitrile, and the like. It should be noted that R-R''' may be virtually any radical which does not interfere or significantly reduce the brightening effect of these dyes.

50 The following are examples of the various brightener classes which are pertinent to this invention.

Class I: Acyldiaminostilbenes

- 55 4,4'-bis(p-methylbenzamido)-2,2'-stilbenedisulfonic acid
- 4,4'-bis(o-ethoxybenzamido)-2,2'-stilbenedisulfonic acid
- 4,4'-bis(2,4-dimethoxybenzamido)-2,2'-stilbenedisulfonic acid
- 4,4'-bis(3-methoxy-2-naphthamido)-2,2'-stilbenedisulfonic acid

Class II: Triazinylaminostilbenes

- 65 4,4'-bis(4,6-dianilino-s-triazin-2-ylamino)-2,2'-stilbenedisulfonic acid
- 4,4'-bis(4-anilino-6-hydroxy-s-triazin-2-ylamino)-2,2'-stilbenedisulfonic acid
- 4,4'-bis[4-anilino-6-bis(2-hydroxyethyl)-amino-s-triazin-2-ylamino]-2,2'-stilbenedisulfonic acid

Class III: Acyldiaminodibenzothiophene dioxide

- 70 Dioxide of 3,7-bis(4-methoxybenzamido)-2,8-dibenzothiophenedisulfonic acid
- Dioxide of 3,7-bis(4-naphthamido)-dibenzothiophenedisulfonic acid

Class IV: Benzimidazoles

- 75 2,2'-ethylenebisbenzimidazolesulfonic acid

## Class V: Triazoles

2-(4-styryl-3-sulfophenyl)-2H-naphtho[1,2]-triazole-5-sulfonic acid

As noted above, the fluorescent textile brighteners are applied simultaneously with the neomycin from aqueous solutions containing the same.

In general, the aqueous solutions containing the fluorescent textile brightener and neomycin may be applied to the textile material by any of the known conventional textile finishing techniques, whereby the material is contacted with these components for a sufficient period of time to fix them on the material. Thus, for example, they may be applied by padding, spraying, submersion, exhaustion or the like. Of these suggested techniques, padding is greatly preferred, in that most finishing plants are adapted to employ this technique, and within certain limits, more uniform control of the process may be achieved.

The sulfonic groups in the fluorescent textile brighteners employable in this invention impart sufficient solubility or dispersibility to permit their application from aqueous media. In addition, these groups contribute to the substantivity of the brighteners on the cellulosic fibers.

As indicated above, it is preferred to apply the neomycin and fluorescent textile brighteners to suitable textile materials containing cellulose and preferably formed cellulosic fabric, by employing conventional padding techniques. Employing such procedure, the textile material is padded through a bath containing neomycin and a suitable fluorescent textile brightener. Excess of the treating solutions are then removed from the textile material to achieve the desired pick-up by passing the impregnated fabric between rollers and thereafter the textile material is dried, preferably at elevated temperatures, as for example temperatures from between 150° F. to 350° F. Caution should be exercised in the employment of elevated temperature to insure that the textile material is not degraded thereby.

The concentration of the neomycin in the treating solution may be varied within wide limits, depending upon the use to which the material is intended. When applied by padding, the solution should contain from approximately 0.0001% to 4% and more by weight of neomycin as is desired in the dried fabric, since in the padding operation the fabric is usually impregnated with from between about 25% to 150% of the weight of the liquid and then dried. When applied by exhausting, the treating solution of neomycin may contain as little as 0.001 micrograms per milliliter of neomycin when highly absorbent cellulosic fibers are treated. From 5 to 500 micrograms of neomycin per milliliter is considered the preferred range for application by exhaustion. For normally prophylactic purposes, sufficient concentration of neomycin may be substantially adhered to base materials from aqueous treating solutions containing from about 1 microgram to about 400 micrograms per milliliter, with commercial limits lying between about 2 and about 200 micrograms per milliliter.

The treating solution should normally contain from approximately 0.001% to 4% and more by weight of the fluorescent brightener as is desired in the dried fabric when applied by padding, since in the padding operation the fabric is usually impregnated with from about 25% to about 150% of the weight of the liquid and then dried.

The concentration of the neomycin applied to the cellulose material may to some extent be varied over wide limits, depending upon the use for which the material is intended. Useful results are obtained when the fabric contains as little as 0.0001% by weight of neomycin on the dry weight of the textile material. The preferred range varies from about 0.001% to 1% by weight of neomycin on the dry weight of the treated fabric. For prophylactic purposes, deposition of from about 0.005 microgram up to 10 micrograms per square centimeter has been found satisfactory, with preferred

commercial ranges lying between about 0.1 and about 6 micrograms per square centimeter.

With respect to the fluorescent organic brightener, useful results are obtained in accordance with the present invention when suitable brightener is present on the fabric in an amount of at least 0.001% though preferably the amount based on the dry weight of the fabric is from between about 0.01 to 0.05%. Concentrations of brightener on the fabric of less than 0.001%, based on the fabric's dry weight, are for the most part impractical.

With respect to formed fabrics, the preferred class of cellulose-containing textile materials contemplated by this invention, they may take any shape, size or form and may clearly include articles which are intended to be reused. Specific illustrations of such articles would include wearing apparel, handkerchiefs, diapers, hand, dish and bath towels, books and book covers, washable cloth toys, dolls and similar playthings, hospital and hotel sheets and pillow cases, hospital and examination room bathrobes, slippers, barbers' and beauticians' cloths and similar articles.

In the subsequent examples and tables of this specification, the test referred to therein for determination of antibacterial activity is a standard one and the treated fabrics are tested by a standard Agar plate method. For evaluating the extent of durability of the antibacterial activity of the textile finish, a convenient test method has been devised on inhibition of the bacterial growth by a piece of textile placed on an Agar plate inoculated with various strains of bacteria. The two commonly used strains are *E. coli* and *S. aureus*, which are strains usually employed in the evaluation of antibacterial agents for various purposes.

Thus, by determining the antibacterial activity of cloth treated by the process of this invention before and after a number of laundering treatments, the effectiveness of the finish may be determined. Durability of the finish is determined by subjecting the treated textile to a series of repeated launderings. The number of times the material may be laundered before antibacterial activity decreases below an effective level will give a measure of the durability of the finish.

In the test for antibacterial activity, discs of treated fabric of a certain size (11.5 millimeters in diameter) are placed on an Agar plate inoculated with the bacterial culture. After two hours contact, the disc is removed and the Agar plate is incubated overnight. The degree of inhibition of growth gives an index of the inhibitory effect of the finish on the cloth. This inhibition is easily observed, since the area where the bacterial growth is inhibited remains clear, whereas the remainder of the area where the bacterial growth has taken place becomes cloudy or opaque. The area under the disc is observed, and in addition, the total diameter of the area larger than that occupied by the disc is observed.

Effective finishes show a clear area at least under the disc with more effectively finished materials giving areas having a diameter greater than that of the disc itself. If the area of inhibition is greater than the area of the disc, the activity is given as the diameter of the clear area in millimeters. Otherwise, a rating of "C" denotes complete inhibition of bacterial growth under the disc; a rating of "P" denotes partial inhibition; an "N" rating denotes no inhibition or activity; and "S" and "VS" denote slight and very slight inhibition. It should be noted that "P" is at least 50 to 75% inhibition under the test fabric.

The whiteness of the treated fabric as reported in subsequent examples and tables is judged by visual observation.

In order that the present invention may be more fully understood, the following examples are given primarily by way of illustration. No details or specific enumerations contained therein should be construed as limitations on the present invention, except as they appear in the

appended claims. All parts and percentages are by weight unless specifically designated otherwise.

#### EXAMPLE 1

125 parts of a solution of neomycin sulfate containing 1% neomycin base was diluted with about five times as much water at room temperature. 0.146 part of 4,4'-bis[4-anilino-6-bis(2-hydroxyethyl)amino-s-triazin-2-ylamino]-2,2'-stilbenedisulfonic acid was added and a precipitate formed. A 1% solution of sodium carbonate was then added with stirring until the precipitate just redissolved (pH of 8-9). This mixture was then diluted with water at room temperature to give a concentration of 0.125% neomycin base and 0.0146% brightener. Bleached 80 x 80 cotton fabric was passed through the above solution, the excess solution was removed by passing the fabric through squeeze rolls to give an 80% expression, and the treated fabric was dried at 225° F. The fabric contained 0.1% neomycin and 0.0117% brightener on the weight of the fabric.

#### EXAMPLE 2

The procedure of Example 1 was used with the substitution of dilute aqueous ammonia for the solution of sodium carbonate. A solution was obtained at a pH of 8-9.

#### EXAMPLE 3

A solution containing 0.125% of neomycin sulfate as the base and 0.014% of 4,4'-bis(2-ethoxybenzoylamino)-2,2'-stilbenedisulfonic acid was prepared using sufficient aqueous ammonia to dissolve the precipitate which formed when the brightener was added to the neomycin solution. Bleached 80 x 80 cotton fabric was treated with the solution as described in Example 1. The treated fabric contained 0.1% of neomycin and 0.011% of brightener on the weight of the fabric.

#### EXAMPLE 4

The procedure of Example 3 was used substituting 0.0027% of 4,4'-bis(2,4-dimethoxybenzoylamino)-2,2'-stilbenedisulfonic acid for the 4,4'-bis(2-ethoxybenzoylamino)-2,2'-stilbenedisulfonic acid. The treated fabric contained 0.1% of neomycin and 0.0022% of the brightener on the weight of the fabric.

#### EXAMPLE 5

The procedure of Example 3 was used substituting 0.0325% of dioxime of 3,7-bis(4-methoxybenzamido)-2,8-dibenzothiophenedisulfonic acid, [4,4'-bis(4-methoxybenzoylamino)2,2'-sulfonylbiphenylsulfonic acid]. The treated fabric contained 0.1% of neomycin and 0.026% of the brightener on the weight of the fabric.

#### EXAMPLE 6

The procedure of Example 5 was used substituting 0.00325% of the same brightener for the 0.0325% used in Example 5. The treated fabric contained 0.1% of neomycin and 0.0026% of the brightener on the weight of the fabric.

#### EXAMPLE 7

125 parts of a solution of neomycin sulfate containing 1% of neomycin base was diluted with water at room temperature to give a concentration of 0.125% neomycin base. Bleached 80 x 80 cotton fabric was passed through the solution, and the excess solution was removed by passing the fabric through squeeze rolls to give an 80% expression. The fabric was dried at 225° F.

#### EXAMPLE 8

The cotton fabrics to which neomycin and brightener had been applied as described in Examples 2-5 and 7 were tested for antibacterial activity. The fabrics were laundered at 140° F. in hard water by a standard procedure using a Laundromat washing machine containing 9 gallons of water with 20 cc. of 10% calcium chloride

and 0.25% neutral soap added. The antibacterial tests were repeated after the 16th and 25th washes.

The results are shown in Table I hereinbelow.

Table I

|                   |  | Zone of Inhibition |           |           |
|-------------------|--|--------------------|-----------|-----------|
|                   |  | Initial            | 16 Washes | 25 Washes |
| <i>S. aureus:</i> |  |                    |           |           |
| Example 7         |  | 17.5               | 12.0      | C         |
| Example 2         |  | 17.0               | VS        | P-C       |
| Example 3         |  | 17.3               | C         | P-C       |
| Example 4         |  | 17.6               | C         | P-C       |
| Example 5         |  | 15.8               | C         | P-C       |
| <i>E. coli:</i>   |  |                    |           |           |
| Example 7         |  | 14.4               | VS        | VS        |
| Example 2         |  | 14.4               | VS        | VS        |
| Example 3         |  | 13.8               | S-P       | VS        |
| Example 4         |  | 15.2               | VS        | VS        |
| Example 5         |  | 14.1               | N-VS      | N-VS      |

#### EXAMPLE 9

The cotton fabrics to which neomycin and brightener had been applied as described in Examples 2-7 were tested for durability of whiteness by washing in hard water as described in Example 8. The whiteness of the fabrics were observed visually by daylight, initially and after 16 and 25 washes. The results of these tests are shown in Table II hereinbelow.

Table II

|           |                            | Whiteness                       |                                 |                                 |
|-----------|----------------------------|---------------------------------|---------------------------------|---------------------------------|
|           |                            | Initial                         | 16 Washes                       | 25 Washes                       |
| Example 7 | Similar to untreated.      | Yellower than initially.        | Yellower than initially.        | Much yellower than initially.   |
| Example 2 | Much better than standard. | V. sl. yellower than initially. | V. sl. yellower than initially. | V. sl. yellower than initially. |
| Example 3 | Better than standard.      | do                              | do                              | Do.                             |
| Example 4 | do                         | do                              | do                              | Do.                             |
| Example 5 | do                         | do                              | do                              | Do.                             |
| Example 6 | SI. better than standard.  | SI. yellower than initially.    | SI. yellower than initially.    | SI. yellower than initially.    |

In order to demonstrate that the pH of the aqueous treating solution is a critical element in producing clear stable solutions, the following illustrative examples are presented.

#### EXAMPLE 10

Five aqueous solutions containing .2% neomycin sulfate had their pH adjusted by the addition of dilute sodium hydroxide to 4.8, 7.0, 8.0, 9.0 and 10.0.

To this was added a solution containing approximately 25% of 4,4'-bis[4-anilino-6-bis(2-hydroxyethyl)amino-s-triazin-2-ylamino]-2,2'-stilbenedisulfonic acid.

The final solutions contained .1% of neomycin sulfate and 0.025% of the anionic brightener identified above.

Only the solutions employing the neomycin sulfate solutions having adjusted pH's of 9 and 10 were clear and stable. Those neomycin sulfate solutions having their pH's adjusted to 4.8, 7.0 and 8.0 showed the presence of substantial amounts of precipitate.

#### EXAMPLE 11

250 parts of cold water were added to 62.5 parts of a 1% solution of neomycin sulfate.

100 parts of water were added to 0.7 part of a solution of 4,4'-bis[4-anilino-6-bis(2-hydroxyethyl)amino-s-triazin-2-ylamino]-2,2'-stilbenedisulfonic acid containing approximately 25% of said compound. The brightener solution was added to the neomycin solution with stirring and 1% of a solution of soda ash was added dropwise with stirring until the solution cleared. The pH was checked at the first point of clarification, which was found to be a value of 8.7.

This solution was then made up to a final volume of 500 cc. so that the solution contained .125% of neomycin and .0375% of 4,4'-bis[4-anilino-6-bis(2-hydroxyethyl)amino-s-triazin-2-ylamino]-2,2'-stilbenedisulfonic acid. The pH of the final volume of this solution was determined to be 8.7.

#### EXAMPLE 12

The above procedure was repeated with the exception that 250 cc. of cold water were added to 6.3 parts of a 1% solution of neomycin sulfate as compared with the 62.5 parts in Example 11.

The pH at the first point of clarification was 8.9.

#### EXAMPLE 13

Approximately 250 parts of cold water were added to 62.5 parts of a 1% solution of neomycin sulfate. The pH of this solution was adjusted to 7.5 with a 1% solution of soda ash.

0.75 part of a 25% solution of 4,4'-bis[4-anilino-6-bis(2-hydroxyethyl)amino-s-triazin-2-ylamino]-2,2'-stilbenedisulfonic acid is diluted with approximately 100 parts of water. The pH of this solution is adjusted to 7.5 by the addition of dilute sulfuric acid. The brightener solution is then added to the solution of neomycin and the total volume adjusted to 500 cc. The pH of the solution is 7.5.

This identical procedure was repeated to produce solutions having pH's of 8, 8.5 and 9, and the compatibility of these solutions at each of these pH levels was noted. The final solutions having pH's of 7.5 and 8 contained substantial precipitate, while that having a pH of 8.5 was turbid. The solution having a pH of 9 was water clear and stable.

#### EXAMPLE 14

Approximately 250 parts of cold water were added to 62.5 parts of a 1% solution of neomycin sulfate. The pH of the solution was adjusted to 9 with a 1% solution of soda ash.

Approximately 100 parts of water were added to 0.75 part of a 25% solution of 4,4'-bis[4-anilino-6-bis(2-hydroxyethyl)amino-s-triazin-2-ylamino]-2,2'-stilbenedisulfonic acid. No pH adjustment was made in the diluted brightener solution. The brightener solution was added to the solution of neomycin with moderate manual stirring and the final volume of the solution adjusted to 500 parts. The resulting solution was stable and water clear and had a pH of 9.

This example points out that the addition of the alkaline brightener solution, which has a pH of 9.75 when employed in conventional and in effective amounts, is in amounts insufficient to affect the pH of the final solution.

While the present invention relates primarily to the finishing of cellulosic containing textile materials with a purifying finish containing neomycin and a fluorescent organic brightener, it will be apparent that other textile treating agents, lubricants, softeners, wetting agents, and

the like may be incorporated into the treating bath, so long as their presence and function do not inhibit or impair the antibacterial finish and its durability and the brightening effects achieved in accordance with this invention.

This application is a continuation-in-part of our pending application Serial No. 771,194, filed November 3, 1958, now abandoned.

We claim:

- 10 1. A process for finishing formed textile fabric containing at least 50% cellulosic fibers to impart a durable antibacterial finish thereto having resistance to discoloration which comprises simultaneously applying thereto an aqueous treating solution having a pH above 8.5 and containing neomycin, an anionic fluorescent brightener containing a sulfonic acid group that is substantive to cellulose fiber, and an alkaline agent, so as to impart at least .0001% of neomycin and at least .001% of said anionic brightener to the finished fabric, and thereafter drying the fabric.
- 15 2. A process according to claim 1, wherein the brightener is an acyldiaminostilbene.
- 20 3. A process according to claim 1, wherein the brightener is a triazinylaminostilbene.
- 25 4. A process according to claim 1, wherein the brightener is an acyldiaminodibenzothiophene dioxide.
- 30 5. A process according to claim 1, in which the neomycin is applied so as to be present on the fabric in an amount of from between .0001 and .1%, based on the dry weight of the fabric, and the anionic fluorescent brightener is present on the fabric in an amount of from between .001 and 0.05%, based on the dry weight of the fabric.
- 35 6. A process according to claim 1, in which the fabric is cotton.
- 35 7. A process according to claim 3, in which the neomycin is applied to the fabric in an amount from between about .01 and .05%, based on the dry weight of the fabric and the anionic brightener is applied to the textile material in an amount from between about .01 and .05%, based on the dry weight of the fabric.
- 40 8. A composition which comprises in aqueous medium, neomycin, at least .001% of an anionic fluorescent brightener containing a sulfonic acid group, and an alkaline agent, said composition being characterized by a pH above 8.5.

#### References Cited in the file of this patent

#### UNITED STATES PATENTS

|    |           |           |       |                |
|----|-----------|-----------|-------|----------------|
| 50 | 2,468,431 | Eberhart  | ----- | Apr. 26, 1949  |
|    | 2,563,493 | Scalera   | ----- | Aug. 7, 1951   |
|    | 2,563,795 | Scalera   | ----- | Aug. 7, 1951   |
|    | 2,567,796 | Ackermann | ----- | Sept. 11, 1951 |
| 55 | 2,763,650 | Ackermann | ----- | Sept. 18, 1956 |
|    | 2,830,011 | Parker    | ----- | Apr. 8, 1958   |

#### OTHER REFERENCES

Dorset: Textile Manufacturer, May 1954, pp. 254-258.